

## UNITED STATES PATENT OFFICE

2,339,242

## COATED SHEET MATERIAL

Allen Abrams and George W. Forcey, Wausau,  
and Charley L. Wagner, Menasha, Wis., as  
signors to Marathon Paper Mills Company,  
Rothschild, Wis., a corporation of Wisconsin

No Drawing. Application August 2, 1940,  
Serial No. 349,767

5 Claims. (Cl. 117—146)

This invention relates to a coated sheet material, having a thermoplastic composition, suitable for the packaging of food products and the like.

An object of the invention is to provide a coated sheet material having a continuous thermoplastic flexible film thereon suitable for packaging of molten food materials such as process cheese, chocolate, candy, jellies and the like, and which coated sheet will remain flexible and pliable upon cooling of the goods packaged therewith.

A further object of the invention is to provide a coated sheet material having a flexible, continuous, thermoplastic coating film thereon suitable for packaging foods and adapted to be in contact with hot or molten foods and which will retain the self-sustaining characteristics as well as flexibility of the film after cooling of the food and will not become brittle, but will adhere to the sheet material in a continuous film.

Still another object of the invention is to provide a sheet material coated with a wax-rubber coating composition so compounded as to provide a continuous flexible film adapted for packaging foods in molten condition, and which will retain flexibility and not become brittle upon cooling of the contents after packaging.

Another object of the invention is to provide a coated sheet material of such character that if the coating should separate from the base sheet, both the base sheet and the coating layer alone are sufficiently strong and self-sustaining so as to be removable separately.

Other and further objects of this invention will be apparent from the following specification wherein further details of the invention are given.

The patents to Abrams et al., Nos. 2,054,112 and 2,054,113, disclose a composition comprising wax and rubber suitable for coating sheet materials. The sheet materials are coated with a hot-melt wax-rubber composition having a viscosity of at least 8,000 seconds (50 cc. measured on a Scott viscosimeter at 90° C.). We have found that when the coated sheet materials made according to these patents are used for packaging hot or molten food products, particularly when such food products are brought into direct contact with the coating composition or film on the sheet material, there is a tendency for the coating on the sheet to soften, and upon cooling the coating film loses its original flexibility and does not retain its original self-sustaining characteristics. On cooling the coating also tends to become brittle, so that when the package is 55

opened, the coating may flake and adhere to the food instead of remaining as a continuous film adhering to the sheet material.

When process cheese or other molten foods are packaged in such coated sheet material, the packages are often placed in refrigerators where they are chilled and brought into a humid room so as to produce condensation of moisture on the surface of the package causing the coating film to separate from the sheet material and remain upon the food about which the sheet is wrapped. If such film does not retain its flexibility as well as its self-sustaining characteristics it will be difficult to remove the film from the food.

In packaging process cheese, for example, in accordance with the method disclosed in Abrams et al. Patent No. 2,077,301, the coated sheet is lined in a wooden box and the like with the film or coating facing the interior of the container. The molten cheese is then poured into contact with the coating, the air is expelled from the package, and the overlapping portions of the wrapper are then hermetically heat-sealed. 20 American process cheese, for example, may be poured into such lined containers at a temperature of about 150 to 160° F. After the package is completed the hot cheese will remain in contact with the coating on the sheet or wrapper 25 for a considerable period of time. In fact, it is the practice of cheese manufacturers after packaging the cheese in such wrapper to store the boxes containing the packaged cheese for about twelve to sixteen hours to permit the cheese to cool. During such time the coating on the sheet is subjected to relatively high temperatures and then to slow cooling. During such time the coating is in softened condition which is desirable in order to cause intimate contact of the coating 30 with the cheese. However, as a result of these severe temperature conditions and slow cooling, the coating material tends to become brittle and loses its flexibility, so that when the package of cheese is opened for use, the sheet material will 35 separate from the coating and leave particles of the composition on the cheese.

It is therefore desirable to modify the composition of wax and rubber as disclosed in the aforementioned patents so that the coating on the sheet will soften sufficiently to permit intimate contact with the food and yet retain its self-sustaining characteristics in spite of the long exposure to heat as well as the slow cooling.

We have discovered after considerable experimentation that these difficulties can be overcome

by adding to the composition a controlled quantity of microcrystalline or amorphous waxes. Any suitable amorphous or microcrystalline waxes may be used for the purpose of our invention. For example, "Barnsdall special wax" sold by the Barnsdall Refinery Company, is satisfactory. Also "Cerese" waxes sold by the Socony Vacuum Company, carnauba, synthetic waxes, hydrogenated vegetable oils such as hydrogenated cottonseed oil, soya bean oil, and castor oil; also hydrogenated animal oils such as fish oils; also hydrogenated waxes such as I. G. wax, also beeswax, candelilla, spermaceti, and wool wax, are suitable. The term "amorphous wax" is intended to include all these substances.

The following is an illustration of a composition suitable for coating sheet materials for use in packaging molten foods such as American process cheese at, say, 150-155° F.

|                                                        | Per cent<br>by weight |
|--------------------------------------------------------|-----------------------|
| Pale crepe rubber                                      | 18                    |
| Amorphous wax—Barnsdall special wax<br>(165° F. M. P.) | 39                    |
| Paraffin wax (120-140° F. M. P.)                       | 43                    |

In compounding the composition the waxes are first melted and maintained at a temperature from about 180 to 220° F. The rubber, preferably in the form of pale crepe sheets, is added in small pieces to the molten wax mixture and stirred until the rubber is completely penetrated by the wax. The mixture is then thoroughly stirred in a Werner-Pfleiderer mixer for about 1½ to 2 hours while the temperature is maintained at around 180 to 190° F. until a uniform homogeneous composition is obtained. As soon as the mixture is entirely smooth it is coated while hot upon any suitable base sheet by any well known means, such as by means of a hot roll or doctor bar. The composition is compounded so as to have a minimum viscosity of 8,000 seconds (50 cc. measured on a Scott viscosimeter at 90° C.). It is important that the viscosity is not lowered below this value during compounding because if this occurs the film produced from the composition will not have the desired self-sustaining characteristics as well as flexibility, pliability, and the like. It is also important that the temperature during the compounding should not be higher than about 200° F. in order not to scorch or burn the rubber, as this will impart an undesirable color and odor to the composition which will be objectionable when used for packaging food products.

The following is an example of a composition coated on a sheet material suitable for packaging molten foods having a higher melting point than American process cheese, e. g. 160-165° F.:

|                               | Per cent<br>by weight |
|-------------------------------|-----------------------|
| Rubber                        | 18                    |
| Ester gum                     | 8                     |
| Amorphous wax (165° F. M. P.) | 44                    |
| Paraffin wax (145° F. M. P.)  | 30                    |

This composition is compounded in a similar manner as the previous example so as to have a viscosity of not less than 8,000 seconds (50 cc. measured on a Scott viscosimeter at 90° C.). The composition is similarly coated on any suitable sheet material by means of a hot roll or doctor blade.

The rubber, or equivalent film-forming constituent, in our composition may range anywhere from about 6 to 50 percent by weight. The paraf-

fin wax or other equivalent crystalline waxy constituent may range anywhere from 94 to 50 percent by weight. According to our invention we combine with the crystalline paraffin wax a controlled proportion of an amorphous or microcrystalline wax anywhere in the range from about 5 to 50 percent by weight of the total paraffin wax used. As previously explained, we have found that the addition of amorphous wax to a composition containing crystalline paraffin wax and rubber, serves to increase the pliability and flexibility of the film after it has been subjected to high temperatures and then cooled slowly over an extended period of time. The film after such treatment also will not crumble or separate from the sheet to which it has been applied.

Our composition may be applied to any suitable sheet material such as Pliofilm, Cellophane (regenerated cellulose), cellulose acetate, ethyl cellulose films, casein sheets, sulphite paper, kraft paper, parchment paper, glassine, metal foil, fabric, rayon, sheets made of synthetic resinous substances, and the like. The composition will not penetrate or saturate the sheet material to which it is applied, but it will remain as a self-sustaining continuous film upon the surface of the sheet and when used for packaging molten or hot foods which are brought in contact with said film, the film will retain its pliability and flexible characteristics so that when the wrapper is peeled from the packaged food the film will adhere to the sheet material and will not become brittle, crumble, or fall apart and thereby contaminate the food in the package. Even if the coating film should separate from the base sheet when wet, the film will retain its strength and elasticity so as to be self-sustaining without crumbling or falling apart. When non-wetting sheet materials are used such as Pliofilm, cellulose acetate, foil, and the like, the coating film will not readily separate when the coated sheet is wet.

The invention is not restricted to the use of rubber in the composition and it is to be understood that any suitable film forming material similar to rubber in its characteristics can be used, such as synthetic rubber, Vistanex (isobutylene polymers), gutta percha, balata, smoked sheet rubber, chlorinated rubbers and the like.

It is to be understood that numerous modifications and changes may be made in our coating composition, and that it is intended to include such modifications within the scope of the appended claims.

We claim:

- 55 1. A coated sheet material suitable for packaging molten food materials such as process cheese and the like which comprises a sheet material having a superficially adherent, self-sustaining, flexible film of tangible thickness formed from a hot melt composition having a viscosity of at least 8,000 seconds (50 cc. measured on a Scott viscosimeter at 90° C.) comprising a uniform homogeneous mixture of 6 to 50% by weight of rubber, 94 to 50% by weight of paraffin wax and an amorphous wax blended with the paraffin wax in amount for the film to have flexibility and self-sustaining characteristics after pouring and slow cooling of hot molten materials in direct contact therewith.
- 60 2. A coated sheet material suitable for packaging molten food materials such as process cheese and the like which comprises a sheet material having a superficially adherent, self-sustaining, flexible film of tangible thickness formed from a hot-melt composition having a
- 65
- 70
- 75

viscosity of at least 8,000 seconds (50 cc. measured on a Scott viscosimeter at 90° C.) comprising a uniform homogeneous mixture of 6 to 50% by weight of rubber, 94 to 50% by weight of paraffin wax and a controlled quantity of an amorphous wax blended with the paraffin wax in amount from 5 to 50% by weight of the paraffin wax, said film having flexibility and self-sustaining characteristics after pouring and slow cooling of hot molten materials in direct contact therewith.

3. A coated sheet material suitable for packaging molten food materials such as process cheese and the like which comprises a regenerated cellulose sheet material having a superficially adherent, self-sustaining, flexible film of tangible thickness formed from a hot-melt composition having a viscosity of at least 8,000 seconds (50 cc. measured on a Scott viscosimeter at 90° C.) comprising a uniform homogeneous mixture of 6 to 50% by weight of rubber, 94 to 50% by weight of paraffin wax and an amorphous wax blended with the paraffin wax in amount for the film to have flexibility and self-sustaining characteristics after pouring and slow cooling of hot molten materials in direct contact therewith.

4. A coated sheet material suitable for packaging molten food materials such as process cheese and the like which comprises a sheet material having a superficially adherent, self-sustaining, flexible film of tangible thickness

5 10 formed from a hot-melt composition having a viscosity of at least 8,000 seconds (50 cc. measured on a Scott viscosimeter at 90° C.) comprising a uniform homogeneous mixture of 6 to 50% by weight of a wax-compatible film-forming constituent selected from the group consisting of natural and synthetic rubber, gutta percha, balata, chlorinated rubber, and isobutylene polymers, 94 to 50% by weight of paraffin wax and an amorphous wax blended with the paraffin wax in amount for the film to have flexibility and self-sustaining characteristics after pouring and slow cooling of hot molten materials in direct contact therewith.

15 20 25 30 5. A coated sheet material suitable for packaging molten food materials such as process cheese and the like which comprises a sheet material having a superficially adherent, self-sustaining, flexible film of tangible thickness formed from a hot-melt composition having a viscosity of at least 8,000 seconds (50 cc. measured on a Scott viscosimeter at 90° C.) comprising a uniform homogeneous mixture of 6 to 50% by weight of rubber, 94 to 50% by weight of paraffin wax and a microcrystalline wax blended with the paraffin wax in amount for the film to have flexibility and self-sustaining characteristics after pouring and slow cooling of hot molten materials in direct contact therewith.

ALLEN ABRAMS.

GEORGE W. FORCEY.

CHARLEY L. WAGNER.